

## UNITED STATES PATENT OFFICE

PAUL RABE, OF LEVERKUSEN-ON-THE-RHINE, GERMANY, ASSIGNOR TO GENERAL ANILINE WORKS, INC., OF NEW YORK, N. Y., A CORPORATION OF DELAWARE

## PROCESS FOR INCREASING THE FASTNESS TO LIGHT OF BASIC DYESTUFFS

No Drawing. Application filed September 20, 1927, Serial No. 220,830, and in Germany August 12, 1926.

In the copending application, Serial No. 190,129, filed May 9, 1927, there are described new molybdenum phosphotungstate compounds obtainable by reduction of the two complex molybdenum phosphotungstic acids of the general formula:



wherein  $n$  stands for one of the numbers 18 and 24 which compounds are soluble in water very easily, are quite stable in air and are convertible into molybdenum phosphotungstate acids by means of oxidizing agents.

The complex molybdenum phosphotungstic acids may be prepared in the following manner, all parts being by weight:

100 parts of sodium tungstate  
25 parts of sodium molybdate

20 are dissolved in 225 parts of water. Thereto 85 parts of phosphoric acid (85%), 115 parts of 19° Bé. hydrochloric acid, and 2 parts of nitric acid are added. The mixture is boiled for about 8 hours and is then allowed to cool 25 slowly, whereby the sodium salt of the acid of the formula:



separates in large crystals. The addition of 30 ammonium salts to the mother liquor causes no turbidity which means that the acid of the formula:



35 is separated quantitatively. By the addition of about 50 parts of ammonium chloride to the filtrate the acid of the formula



40 is salted out.

The reduction may be effected in the usual way, for instance in aqueous solution by means of sulfuric acid, bisulfite, hydro-sulfite, the lower oxidation products of 45 molybdenum, grape sugar or the like, and from the reduced solution the new products may be precipitated, for instance with hydro-chloric acid.

Now I have found that by subjecting materials dyed by means of basic dyestuffs to a

subsequent treatment with these compounds, the fastness to light of the dyeings is considerably increased. For this purpose I prefer to treat the dyed materials with diluted aqueous solution of one of the above described 55 reduction products.

The following example will illustrate my invention without limiting it thereto.

## Example

A 1% dyeing of rhodamine B-Extra (compare colour Index 1924, page 190, No. 749) on a tannin-antimony mordant is treated for half an hour at a temperature of about 50–60° C. with a solution containing from 0.1 to 0.2 60 grams of the product obtainable by reduction of the molybdenum phosphotungstic acid of the formula



in 70 100 cc. of water and dried without rinsing. The dyeing is considerably more fast to light than the untreated dyeing.

I claim:

1. A process for increasing the fastness to 75 light of dyeings with basic dyestuffs which consists in treating the dyeings with a compound obtainable by reduction of a complex molybdenum phosphotungstic acid wherein  $n$  represents one of the numbers 18 and 24. 80

2. A process for increasing the fastness to 85 light of dyeings with basic dyestuffs which consists in treating the dyeings with an aqueous solution of a compound obtainable by reduction of a complex molybdenum phosphotungstic acid wherein  $n$  represents one of the numbers 18 and 24.

3. A process for increasing the fastness to 90 light of dyeings with basic dyestuffs which consists in treating the dyeings with an aqueous solution of the compound obtainable by reduction of a complex molybdenum phosphotungstic acid wherein  $n$  represents one of the numbers 18 and 24 and then drying without rinsing.

4. A process for increasing the fastness to 95 light of dyeings with basic dyestuffs which consists in treating the dyeings with an aqueous solution of the compound obtainable 100

by reduction of the complex molybdenum phosphotungstic acid of the formula



5 and then drying without rinsing.

5. Materials dyed by means of a basic dye-stuff and subsequently treated with a product obtainable by reduction of a complex molybdenum phosphotungstic acid wherein

10  $n$  represents one of the numbers 18 and 24.

6. Materials dyed by means of a basic dye-stuff and treated subsequently with an aqueous solution of the compound obtainable by reduction of the molybdenum phospho-tungstic acid of the formula



In testimony whereof I have hereunto set my hand.

20 PAUL RABE.

25

#### Certificate of Correction

Patent No. 1,736,835.

Granted November 26, 1929, to

PAUL RABE

It is hereby certified that error appears in the printed specification of the above numbered patent requiring correction as follows: Page 1, lines 79, 86, and 94, claims 1, 2, and 3, and page 2, line 9, claim 5, after the word "acid" insert

*of the general formula:  $n(WO_3 + MoO_3) \cdot P_2O_5 \cdot 3H_2O$*

and that the said Letters Patent should be read with this correction therein that the same may conform to the record of the case in the Patent Office.

Signed and sealed this 24th day of December, A. D. 1929.

[SEAL]

M. J. MOORE,  
*Acting Commissioner of Patents.*

55

60

65

by reduction of the complex molybdenum phosphotungstic acid of the formula



5 and then drying without rinsing.

5. Materials dyed by means of a basic dye-stuff and subsequently treated with a product obtainable by reduction of a complex molybdenum phosphotungstic acid wherein

10  $n$  represents one of the numbers 18 and 24.

6. Materials dyed by means of a basic dye-stuff and treated subsequently with an aqueous solution of the compound obtainable by reduction of the molybdenum phospho-tungstic acid of the formula



In testimony whereof I have hereunto set my hand.

20 PAUL RABE.

25

#### Certificate of Correction

Patent No. 1,736,835.

Granted November 26, 1929, to

PAUL RABE

It is hereby certified that error appears in the printed specification of the above numbered patent requiring correction as follows: Page 1, lines 79, 86, and 94, claims 1, 2, and 3, and page 2, line 9, claim 5, after the word "acid" insert

*of the general formula:  $n(WO_3 + MoO_3) \cdot P_2O_5 \cdot 3H_2O$*

and that the said Letters Patent should be read with this correction therein that the same may conform to the record of the case in the Patent Office.

Signed and sealed this 24th day of December, A. D. 1929.

[SEAL]

M. J. MOORE,  
*Acting Commissioner of Patents.*

55

60

65